# EUROPEAN PATENT SPECIFICATION

(11) **EP 3 365 121 B1**
(45) Date of publication and mention of the grant of the patent: **10.04.2019**
(21) Application number: 16707614.0
(22) Date of filing: 08.01.2016
(51) Int. Cl.: B21C 23/20, B21C 23/32

(54) **METHOD OF PRODUCTION OF HIGH-PRESSURE SEAMLESS CYLINDER FROM CORROSION-RESISTANT STEEL**
VERFAHREN ZUR HERSTELLUNG EINES NAHTLOSEN HOCHDRUCKZYLINDERS AUS EDELSTAHL
PROCÉDÉ DE FABRICATION D'UN CYLINDRE HAUTE PRESSION SANS JOINTURE EN ACIER INOXYDABLE

(30) Priority: 03.12.2015 CZ 20150855
(43) Date of publication of application: 29.08.2018
(73) Proprietor: VÍTKOVICE CYLINDERS a.s., 706 00 Ostrava-Vítkovice (CZ)
(72) Inventor: KUCERA, Pavel, 73911 Frydlant nad Ostravici (CZ); HOFRIK, Petr, 70800 Ostrava-Poruba (CZ); PIJANOWSKI, Tomas, 70030 Ostrava-Hrabuvka (CZ)
(74) Representative: Rylkova, Iva
(86) International application number: PCT/CZ2016/050001
(87) International publication number: WO 2017/092721

(56) References cited:
- EP-A1- 2 703 454
- CS-B1- 243 247
- US-A- 4 147 639

## Description

### Technical Field

The invention relates to the field of material forming, namely the method of production of high-pressure cylinder from corrosion-resistant steel using the method of hot backward extrusion solved completely specifically for the possibility to obtain high-pressure seamless cylinder not showing hydrogen embrittlement and inner surface corrosion.

### Background Art

High-pressure seamless steel cylinders are currently produced using the method of backward extrusion and drawing utilizing the process according to the CZ pat. 243247.

When using the procedure according to the CZ patent 243247, steel blanks are first cut from billets of square or circular section. The steel blanks are heated in an induction furnace to the output temperature of 1000 to 1250 °C, after which they are robotically transposed into a descaling device where a high-pressure water jetting is performed to remove the scales from the surface of blanks. Then each individual blank is inserted by stacker into an extrusion press, where it is upset and backward extruded. The backward extrusion process is realized in two steps. During the first step, the blank is inserted into a die with a vertically moving ram, cylindrical insert, and piercing mandrel fitted with a piercing head, where a thick-walled hollow semi-product, which is smooth inside without protrusions or bumps, is produced by means of extrusion from the blank. At the end of extrusion in the extrusion press, bottom is pressed in the semi-product basically to the final thickness, however the semi-product has larger diameter than the final product. After completion of the backward extrusion in the extrusion press, the semi-product is robotically removed from the extrusion press, turned by 90°, and seated in this position into the horizontal drawing press, where the second step of forming, which is backward drawing, will take place. During this second step, the semi-product is put on a drawing mandrel with the already final inner diameter of the cylinder, after which it is extruded through a stripper ring and roller cartridges fitted with reduction rollers. The semi-product on the mandrel is rolled, in which process reshaping of the semi-product wall thickness by approximately 25 % to 85 % will take place, and the semi-product will acquire the desired outer and inner diameter. In addition, the rest of scales will fall off. After the semi-product passing through the stripper ring and the roller cartridges, insertion of the semi-product bottom into a sizing die is performed, thus forming the final shape of the cylinder bottom. Then, in the course of backward movement of the drawing mandrel, the semi-product is pulled off from the drawing mandrel with the help of stripping jaws. The stage of the semi-product processing by rolling is mentioned in the Utility model CZ U 20492. After final forming by rolling, the hollow semi-products are aftercooled with air and subsequently necked, i.e. closed by means of rotary forming to create a steel cylinder of typical geometry.

Disadvantage of the existing procedures of production of high-pressure seamless cylinders is the fact that they do not allow production of cylinders from corrosion-resistant steels using the method of backward extrusion and drawing, because the corrosion-resistant material degrades when conventional method of backward extrusion and drawing is used and it is impossible to produce safe high-pressure seamless cylinder from it.

Currently there are also procedures that allow producing high-pressure cylinders from corrosion-resistant pipes. These are procedures in which necking of pipe segment is performed on both sides. In a seamless form, however, only double-necked cylinders of a simple shape can be manufactured with these procedures, because they do not allow seamless closure of the bottom. Cylinders of different types of alloys such as chrome-molybdenum can also be produced using these procedures. However, because it is not possible to produce sufficiently thin-walled tubes as the starting semi-product for these procedures, all such pressure bottles made using production methods based on pipes have thick-walled structure, and thus they have considerable disadvantage in a very big mass. Especially in the case of bigger volumes, such big weight of cylinders complicates handling, storage, and transportation. Existing thick-walled cylinders have another disadvantage in low strength.

In the steel industry, the use of water glass is known in the field of foundry practice for protection of casting moulds against damage.. In this field, the inner surface of the casting mould is sometimes provided with a coating of water glass so that this coating could prevent direct contact of molten metal with the mould surface and thereby increase the service life of the mould. This coating is resistant to high temperatures used in the foundry practice. Water glass is used in the foundry industry also as a cementing component for the production of foundry moulds of sand.

### Disclosure of Invention

The above-mentioned disadvantages are eliminated by the invention. New method of manufacturing seamless high-pressure cylinder from corrosion-resistant steel is designed allowing the production of thin-walled seamless version of the cylinder from corrosion-resistant steel even for larger and high-volume high-pressure cylinders.

The invention starts from the existing method of manufacturing seamless high-pressure cylinders. The starting part in the form of a steel blank is heated in an induction furnace and then inserted into an extrusion press where it is upset and backward extruded in two steps. From this, during the first step, the blank is inserted into a die with a cylindrical insert and a vertically moving piercing tool, and here it is moulded by means of extrusion until a thick-walled hollow semi-product having an inner cavity, walls and bottom is moulded from it. After that, the semi-product is removed from the extrusion press, turned by 90°, and seated in this position into a horizontal drawing press, where the second step of forming, which is backward drawing, takes place. During this second step, the semi-product is put on a drawing mandrel with the diameter corresponding to the desired final inner diameter of the produced cylinder, while in this drawing press, the semi-product is extruded through a stripper ring and roller cartridges fitted with reduction rollers by means of which it is rolled on the mandrel. This rolling is performed so long until the semi-product acquires the desired outer and inner diameter corresponding to the required final dimensions of the produced cylinder. Then the final shape of the cylinder bottom is formed by insertion of the semi-product bottom into a sizing die and subsequently, in the course of the backward movement of the drawing mandrel, the semi-product is pulled off from the drawing mandrel with the help of stripping jaws and is aftercooled. Finally, the semi-product manufactured in this way is necked, by which the shape of the manufactured cylinder is finished. The essence of the new solution according to the invention is that even before heating in the induction furnace, at least 85 % of the blank surface is coated with coating from material based on water glass with thickness of 20 to 150 µm, this coating is cured by drying at the temperature of 15 to 60 °C and only after this curing, the blank is subjected to heating in the induction furnace.

The material based on water glass is applied to the blank for example by spraying with nozzles or brushing in the form of water glass suspension. The water glass suspension stands here for suspension containing 20 to 40 % w. w. of sodium silicate or potassium silicate or mixture of these silicates, and 80 to 40 % w. w. of water, while in the case of presence of admixtures such as borosilicates and/or corrosion inhibitors, these admixtures are contained in the amount of maximum 20 % w. w.

The blank with coating from material based on water glass is heated in the induction furnace to the temperature of 1180 °C to 1260 °C.

Then, when the blank with coating is heated up in the induction furnace, the blank with coating is taken out of here, and during persistence of its temperature of minimum 1110 °C, it is inserted into the extrusion press, preferably without performing water descaling between the removal from the induction furnace and insertion into the extrusion press.

During the first step of mechanical working, in the course of piercing, the coating of material based on water glass is broken to pieces by purposeful pushing of the piercing tool to the blank, while it is cracking off during extrusion in the extrusion press until at least its major part is removed, meant as thickness of layer.

Then, when the final shape of the cylinder is formed from the semi-product, the leftovers of coating based on water glass are preferably removed from the surface of the semi-product by pressure blasting of its outer as well as inner surface with abrasive.

The blank is made preferably from corrosion-resistant steel while the resulting cylinder is made as a seamless cylinder in the volume range from 5 litres up to 260 litres, as a single necked or double-necked cylinder for any volume within the said range.

Thin walled seamless high-pressure cylinders of the abovementioned volumes are preferably manufactured with the help of this invention. In the second step of forming, the semi-product wall is pressed to the thickness of 2 to 21.5 mm.

The invention is utilizable for manufacturing of seamless high-pressure cylinders. It makes possible to manufacture these cylinders from corrosion-resistant steel and that in the corrosion-resistant version, even for larger and high cylinder volumes from 5 to 260 litres. The invention makes possible to manufacture these cylinders in the thin-walled version from significantly wider range of high-strength corrosion-resistant steels than the existing methods. Using this invention, substantial reduction of the mass of high-pressure cylinders is achieved as compared to the present state of art, and savings of material for their production. The seamless thin-walled version with these volumes was not possible so far. The cylinders according to the invention exhibit high mechanical resistance as well as pressure resistance. They have relatively very low mass, which as compared to the present state of art facilitates manipulation, storage, as well as transport. As compared to cylinders currently manufactured for example for scuba diving, respirators, for calibration gases etc., the cylinders according to the invention are by as much as two thirds lighter. The option to use corrosion-resistant steel for the production makes possible to use these cylinders even for raw natural gas and for gases and mixtures that in the case of existing cylinders from common chrome-molybdenum steel are causing hydrogen embrittlement and accelerated corrosion when reacting with the gas under high pressure.

### Brief Description of Drawings

The invention is illustrated using drawings, where:
Fig. 1 shows the blank with applied coating of water glass in cross-section,
Fig. 2 shows the phase of curing of the coating on the blank,
Fig. 3 shows the phase of relocation of the blank from the induction furnace directly into the extrusion press, and
Fig. 4 A, B shows process of pressing of the blank in the extrusion press, from which A shows the phase of extrusion of the future cylinder cavity in the blank and B shows the subsequent phase of breaking and falling off of the coating from the semi-product during pressing.

### Best Mode for Carrying Out the Invention

Example of embodiment of the invention is visually demonstrated with the help of Figs. 1 to 4 and the hereinafter-described method of production of corrosion-resistant high-pressure seamless cylinder for storage, transport, and use of natural gas.

Parts of the size needed for the manufacture of cylinders of the produced volume are first cut from billets of corrosion-resistant steel having square or circular section. Each individual part, i.e. the starting steel blank 1, is on at least 85 % of its surface coated with coating 2 from material based on water glass. The thickness of applied layer is 20 to 150 µm. Suspension usually called water glass is used as the material based on water glass. For the purposes of the invention, the suspension based on water glass stands for suspension containing 20 to 40 % w. w. of sodium silicate or potassium silicate or their mixture and 80 to 40 % w. w. of water. Admixtures of borosilicates and corrosion inhibitors such as hexamine, fenylethylamine, phosphates, etc. and/or possible other admixtures can be contained provided they do not exceed the amount of 20 % w. w. in the suspension.

Examples of materia! composition of the suspension are given below.

**Suspension I**

| Material | weight % in the suspension |
|---|---|
| Silicates (sodium or potassium silicate or their mixture) | 20 |
| Water | 80 |
| Admixtures | 0 |

**Suspension II**

| Material | weight % in the suspension |
|---|---|
| Silicates (sodium or potassium silicate or their mixture) | 40 |
| Water | 60 |
| Admixtures | 0 |

**Suspension III**

| Material | weight % in the suspension |
|---|---|
| Silicates (sodium or potassium silicate or their mixture) | 30 |
| Water | 60 |
| Admixtures (borosilicates and corrosion inhibitors in quantities 1:1) | 10 |

**Suspension IV**

| Material | weight % in the suspension |
|---|---|
| Silicates (sodium or potassium silicate or their mixture) | 40 |
| Water | 40 |
| Admixtures (borosilicates and unidentified admixtures) | 20 |

This coating 2 can be applied by brushing or spraying. After the application, the coating is let to dry at the temperature of 15 to 60 °C until curing. Sufficient curing will not take place in the case of curing below the temperature of 15 °C, so that unwanted cracking and falling-off of the coating 2 layer would take place during subsequent heating in the induction furnace. In the case of curing above 60 °C, unwanted cracking of the coating 2 will take place as soon as during drying. During curing within the said range, creation of homogenous layer acting as a protective jacket on the surface of the blank 1 takes place. For the drying process or after it, the blank 1 is placed into the induction furnace, where it is heated up by gradual heating to the temperature of 1180 °C to 1260 °C. During heating, neither high-temperature oxidation of the surface of blanks 1 contained in the induction furnace nor forge welding of more pieces of blanks 1, imminent in the case of heating without the coating 2, takes place. The heated up blank 1 with the coating 2 is removed from the induction furnace by robotic feeder 3 and immediately after removal from the induction furnace it is inserted into a die 4 of extrusion press without significant cooling down, with continuation of its temperature of at least 1110°C.

When compared with the process used until now, the step of descaling by water jetting of scale, which is always performed during the existing process between the removal from the induction furnace and insertion into the extrusion press, is skipped. Skipping of the up to now necessary step of water jetting of scale is very significant, because this is preventing cooling down by more than 80 °C, thus eliminating formation of temperature gradient and temperature fluctuations that are typical during the clearing of high-temperature-heating generated scale by means of high-pressure water jet descaling. In addition, the possibility of precise control of the blank 1 temperature is achieved by skipping the descaling.

In the extrusion press, the blank 1, and later the semi-product 5 created from it, is upset and backward extruded in two steps. From this, during the first step, the blank 1 is placed at the bottom 6 of the extrusion press die 4 and here it is pressed by vertically moving ram ended with a piercing mandrel constituting the piercing tool 7. The blank 1 is moulded here by means of extrusion until a thick-walled hollow semi-product 5 having an inner cavity, walls, and bottom is moulded from it, as shown on Figs. 4 A, B. During this first step of mechanical working, in the course of piercing, the coating 2 of material based on water glass is broken to pieces by pushing of the piercing tool 7 to the blank 1 and the semi-product 5 made of it, the coating 2 cracks off, and approximately all this coating 2 is removed during extrusion in the extrusion press. During extrusion, the water glass admixtures will make their way from the coating 2 into the surface layer of the semi-product 5 to the depth of maximum 10 µm, these leftovers are removed later by blasting. The aforementioned extrusion takes place during continuation of the semi-product 5 temperature at 1100 to 1200 °C. Homogenous moulding of the first semi-product 5 does not take place and transversal cracks appear on the semi-product 5 body at a lower temperature. On the contrary, when exceeding the temperature above 1200 °C, oxidation of primary austenitic grains occurs and so called burning out of the material takes place and hence its irreversible degradation. Without using the coating 2, the semi-product 5 could not be extruded and drawn to the required shape, or the corrosion-resistant steel could not be used as the material and/or the result could not lead to the production of the thin-walled seamless high-pressure cylinder of required mechanical and pressure strength.

After completion of processing in the extrusion press, the semi-product 5 is removed from the extrusion press, turned by 90°, and seated in this position into a horizontal drawing press, where the second step of forming in terms of backward drawing takes place. During this second step, the semi-product 5 is put on a drawing mandrel having the diameter corresponding to the desired final inner diameter of the produced cylinder, and in this drawing press, the semi-product 5 is extruded through a stripper ring and roller cartridges fitted with reduction rollers by means of which it is rolled on the mandrel. Rolling is performed so long until the semi-product 5 acquires the required outer and inner diameter. Then the final shape of the cylinder bottom is formed by insertion of the semi-product 5 bottom into a sizing die and subsequently, in the course of the backward movement of the drawing mandrel, the semi-product 5 is pulled off from the drawing mandrel with the help of stripping jaws, aftercooled, and subsequently necked by already known method by means of rotary forming or die forging process. The shape of the manufactured cylinder is finished in this way.

Leftovers of the water glass based coating 2 are removed from the surface of the semi-product 5 by pressure blasting of its outer as well as inner surface with abrasive for example of steel-shot and cast-iron grit.

Corrosion-resistant seamless pressure cylinders in the volume range from 5 litres up to 260 litres can be manufactured using the method according to the invention for any volume within the said range as single necked or double-necked cylinders. In the second step of forming, the invention allows pressing the semi-product 5 wall even to the thickness of a thin-walled cylinder without loss of qualitative properties of the manufactured cylinder. The semi-product 5 wall is pressed even to the thickness of 2 to 21.5 mm. In so doing, the cylinder wall thickness is selected in concrete terms within the above said range depending on the required cylinder volume, pressure for which the cylinder is designated, and requirements for qualitative properties and mechanical strength of the cylinder.

Figures Fig. 1 to 4 illustrate only the steps related directly to the new steps of the process of production of the cylinder according to the invention. The other steps and processes that are already known in this field and are described in the Background Art paragraph do not need to be illuminated using figures.

## Claims

1. Method of production of high-pressure seamless cylinder, in which the starting steel blank (1) is heated in an induction furnace and then inserted into an extrusion press where it is upset and backward extruded in two steps, from which during the first step, the blank (1) is inserted into a die (4) with a vertically moving piercing tool (7), and here it is moulded by means of extrusion until a thick-walled hollow semi-product (5) having an inner cavity, walls and bottom is moulded from it, after which this semi-product (5) is removed from the extrusion press, turned by 90°, and seated in this position into a horizontal drawing press, where the second step of forming in terms of backward drawing takes place, when during this second step, the semi-product (5) is put on a drawing mandrel having the diameter corresponding to the required final inner diameter of the produced cylinder, and in this drawing press, the semi-product (5) is extruded through a stripper ring and roller cartridges fitted with reduction rollers by means of which it is rolled on the mandrel, while this rolling is performed so long until the semi-product (5) acquires the required outer and inner diameter, after which the final shape of the cylinder bottom is formed by insertion of the semi-product (5) bottom into a sizing die and subsequently, in the course of the backward movement of the drawing mandrel, the semi-product (5) is pulled off from the drawing mandrel with the help of stripping jaws, aftercooled, and subsequently necked, by which the shape of the manufactured cylinder is finished, **characterized by that** the starting blank (1) is made from corrosion-resistant steel and even before heating in the induction furnace, the blank (1) is coated on at least 85 % of its surface with coating (2) from material based on water glass with thickness of 20 to 150 µm, this coating (2) is cured by drying at the temperature of 15 to 60 °C and only after this curing, the blank (1) is subjected to heating in the induction furnace.

2. Method of production of high-pressure seamless cylinder from corrosion-resistant steel according to claim 1, **characterized by that** the material applied to the blank (1) for example by spraying or by brush consists of suspension containing 20 to 40 % w. w. of sodium silicate or potassium silicate or mixture of these silicates, and 40 to 80 % w. w. of water, while in the case of presence of admixtures such as borosilicates and/or corrosion inhibitors, the admixtures are contained in the amount of maximum 20 % w. w.

3. Method of production of high-pressure seamless cylinder from corrosion-resistant steel according to claims 1 and 2 **characterized by that** the blank (1) with the coating (2) from material based on water glass is heated in the induction furnace to the temperature of 1180 °C to 1260 °C.

4. Method of production of high-pressure seamless cylinder from corrosion-resistant steel according to any of claims 1 to 3, **characterized by that** after the blank (1) with coating (2) is heated up in the induction furnace, the blank (1) with coating (2) is taken out of here and during persistence of its temperature of minimum 1110 °C, it is inserted into the extrusion press without performing water jetting of scale between the removal from the induction furnace and insertion into the extrusion press.

5. Method of production of high-pressure seamless cylinder from corrosion-resistant steel according to any of claims 1 to 4, **characterized by that** during the first step of mechanical working, in the course of piercing, the coating (2) of material based on water glass is broken to pieces by pushing of the piercing tool (7) to the blank (1) and the coating (2) cracks off during extrusion in the extrusion press until at least its predominant part is removed.

6. Method of production of high-pressure seamless cylinder from corrosion-resistant steel according to claim 5, **characterized by that** after the final shape of the cylinder is formed from the semi-product (5), the leftovers of coating (2) based on water glass are removed from the surface of the semi-product (5) by pressure blasting of its outer as well as inner surface.

7. Method of production of high-pressure seamless cylinder from corrosion-resistant steel according to any of claims 1 to 6, **characterized by that** the blank (1) is made of corrosion-resistant steel while the resulting cylinder is made as a seamless cylinder in the volume range from 5 litres up to 260 litres, as a single necked or double-necked cylinder for any volume within the said range.

8. Method of production of high-pressure seamless cylinder from corrosion-resistant steel according to claim 7, **characterized by that** in the second step of forming, the semi-product (5) wall is pressed to the thickness of 2 to 21.5 mm.

## Patentansprüche

1. Verfahren zur Herstellung eines nahtlosen Hochdruckzylinders aus einem korrosionsbeständigem Edelstahl, wobei ein Stahlzuschnitt (1) im Induktionsofen erwärmt, anschließend in eine Fließpresse zur Anstauchung und zum rückwertigen Fließpressen in zwei Schritten hineingelegt wird, wo während des ersten Schrittes der Zuschnitt (1) in eine Matrix (4) mit vertikal beweglichem Lochwerkzeug (7) hineingelegt und hier mittels des Fließpressens solange gepresst wird, bis ein grobwändiger Rohling mit einem innerem Hohlraum, mit Wänden und mit Boden gefertigt wird, wonach dieser Rohling (5) von der Fließpresse entnommen, um 90° verdreht, und in dieser Position in eine horizontale Ziehpresse, wo der zweite Schritt in Form vom rückwärtigen Ziehpressen verläuft, eingesetzt wird, wo im Verlauf dieses zweiten Schrittes der Rohling auf einen Ziehdorn mit Durchmesser, der dem gewünschten endgültigen Innendurchmesser des Zylinders entspricht, aufgesteckt wird und in dieser Ziehpresse der Rohling (5) durch einen Abstreifring und mehrere Rollenkassetten mit Reduktionsrollen fließgepresst, mit deren Hilfe er auf dem Dorn gewalzt wird, wobei dieses Walzen so lange läuft, bis der Rohling (5) den gewünschten Außen- und Innendurchmesser erhält, wonach durch Eindrücken des Rohlingsbodens (5) in ein Kalibriergesenk, die endgültige Form des Zylinders ausgeformt wird, und nachfolgend, im Verlauf der Rückbewegung des Ziehdorns, der Rohling (5) vom Ziehdorn mit Hilfe von Abstreifbacken zurückgezogen wird, **dadurch gekennzeichnet, dass** der Ausgangszuschnitt (1) aus dem korrosionsbeständigem Edelstahl gefertigt und noch vor der Erwärmung im Induktionsofen auf mindestens 85 % der Oberfläche mit einer Beschichtung (2) auf Wasserglasbasis mit einer Dicke von 20 bis 150 µm versehen wird, diese Beschichtung (2) durch Trocknen bei einer Temperatur von 15 bis 60°C gehärtet wird, und erst nach dieser Aushärtung der Zuschnitt (1) einer Erwärmung im Induktionsofen unterzogen wird.

2. Verfahren zur Herstellung eines nahtlosen Hochdruckzylinders aus Edelstahl nach Anspruch 1, **dadurch gekennzeichnet, dass** das Material, mit welchem der Zuschnitt, zum Beispiel mit Hilfe von Anspritzen oder mit einem Pinsel beschichtet wird, aus einer Suspension mit 20 bis 40 Gewichtsprozent von Natriumsilikat oder Kaliumsilikat oder einer Mischung der genannten Silikaten und 40 bis 80 Gewichtsprozent Wasser besteht, wobei im Falle des Vorhandenseins der Begleitstoffen, wie z.B. Borosilikatenglas und/oder Korrosionsinhibitoren, die Begleitstoffe in einer Menge von höchstens 20 Gewichtsprozent enthalten sind.

3. Verfahren zur Herstellung eines nahtlosen Hochdruckzylinders aus Edelstahl nach den Ansprüchen 1 und 2, **dadurch gekennzeichnet, dass** der Zuschnitt (1) mit Beschichtung (2) von Material auf Wasserglasbasis in einem Induktionsofen auf eine Temperatur von 1180°C bis 1260°C erwärmt wird.

4. Verfahren zur Herstellung eines nahtlosen Hochdruckzylinders aus Edelstahl nach einem der Ansprüche 1 bis 3, **dadurch gekennzeichnet, dass** nachdem der Zuschnitt (1) mit der Beschichtung (2) im Induktionsofen erwärmt wird, wird er aus dem Ofen entnommen und während seine Temperatur von mindestens 1110°C beibehalten wird, der Zuschnitt (1) mit der Beschichtung (2) in eine Fließpresse eingelegt wird, ohne dass zwischen der Entnahme aus dem Induktionsofen und dem Einlegen in die Fließpresse eine Zunderbeaufschlagung durchgeführt wurde.

5. Verfahren zur Herstellung eines nahtlosen Hochdruckzylinders aus Edelstahl nach einem der Ansprüche 1 bis 4, **dadurch gekennzeichnet, dass** im Verlauf des ersten Umformungsschrittes, das heißt des Lochstanzens, durch Drücken des Stanzwerkzeugs (7) die Beschichtung (2) von Material auf Wasserglasbasis zerstückelt und in der Fließpresse abgebrochen wird, bis wenigstens der größte Teil davon entfernt wird.

6. Verfahren zur Herstellung eines nahtlosen Hochdruckzylinders aus Edelstahl nach Anspruch 5, **dadurch gekennzeichnet, dass** nachdem die endgültige Form des Zylinders aus dem Rohling (5) ausgebildet wird, die Reste der Beschichtung (2) auf der Basis von Wasserglas von der äußeren und inneren Oberfläche des Rohlings durch Druckspritzverfahren entfernt werden.

7. Verfahren zur Herstellung eines nahtlosen Hochdruckzylinders aus Edelstahl nach einem der Ansprüche 1 bis 6, **dadurch gekennzeichnet, dass** der Rohling (1) aus dem korrosionsbeständigen Edelstahl gefertigt wird, wobei das endgültige Zylinder als nahtloses Zylinder im Volumenbereich von 5 bis 260 Liter, für ein beliebiges Volumen innerhalb des genannten Bereichs, mit einem einfachen oder Doppelstutzen hergestellt wird.

8. Verfahren zur Herstellung eines nahtlosen Hochdruckzylinders aus Edelstahl nach Anspruch 7, **dadurch gekennzeichnet, dass** im Verlaufe des zweiten Umformungsschrittes die Wand des Zylinders (5) auf eine Dicke von 2 bis 21,5 mm gepresst wird.

## Revendications

1. Procédé de fabrication du cylindre haute pression sans jointures en acier inoxydable, pendant lequel le découpage (1) en acier est chauffé dans un four à induction, puis introduit dans une presse à filer ou il est écrasé et refilé à nouveau en deux étapes, pendant la première étape, le découpage (1) en acier étant déposé dans une matrice (4) avec un outil vertical mobile à perforer (7) ou il est filé jusqu'à ce qu'il devient un semi-produit (5) creux à parois épaisses et avec une cavité intérieure, des parois et un fond, ensuite, ce semi-produit (5) est retiré de la presse à filer et tourné de 90°, puis positionné dans une presse à brocher horizontale ou la seconde étape de façonnage par brochage arrière se déroule, et pendant cette seconde étape, le semi-produit (5) est introduit sur une broche dont le diamètre correspond au diamètre final requis du cylindre à fabriquer, le semi-produit (5) étant passé, dans cette presse à brocher à travers un anneau de grattage et des cassettes à rouleaux munies de rouleaux réducteurs au moyen desquels le semi-produit est roulé, ledit laminage étant effectué jusqu'à ce que le semi-produit (5) obtienne le diamètre interne et le diamètre externe souhaités, puis, en poussant le fond du semi-produit (5) dans une matrice de calibrage, la forme finale est façonnée et pendant le mouvement arrière de la broche, le semi-produit (5) est retiré de la broche à l'aide de mâchoires de grattage, refroidi et muni de goulot, ce qui achève la fabrication de la forme du cylindre, **caractérisé en ce que** le découpage (1) initial est fait en acier inoxydable et avant de passer dans le four à induction, le découpage (1) est traité, sur au moins 85% de sa surface, par un revêtement (2) en matériau à base de verre soluble d'une épaisseur de 20 à 150 µm, ce revêtement (2) se solidifie par séchage à une température de 15 à 60 °C et ce n'est qu'après dudit séchage que le découpage (1) est soumis à l'échauffement dans le four à induction.

2. Procédé de fabrication du cylindre haute pression sans jointures en acier inoxydable selon la revendication 1, **caractérisé en ce que** le matériau déposé sur le découpage (1), par exemple par pulvérisation ou au pinceau, forme des suspensions contenant de 20 à 40% en poids de silicate de sodium ou de silicate de potassium ou du mélange de ces deux silicates de 40 à 80% en poids de l'eau, en cas de présence d'adjuvants comme par exemple des borosilicates et/ou d'inhibiteur de corrosion, le contenu de ces additifs constituant au plus 20% en poids.

3. Procédé de fabrication du cylindre haute pression sans jointures en acier inoxydable selon les revendications 1 et 2, **caractérisé en ce que** dans le four à induction, le découpage (1) avec le revêtement (2) en matériau à base de verre soluble est chauffé à une température de 1180 °C à 1260 °C.

4. Procédé de fabrication du cylindre haute pression sans jointures en acier inoxydable selon les revendications 1 a 3, **caractérisé en ce qu'**après l'échauffement du découpage (1) avec le revêtement (2) dans le four à induction, il en est sorti et si sa température d'au moins 1110°C perdure, le découpage (1) avec le revêtement (2) est introduit dans la presse à filer sans qu'un soufflage d'écailles soit effectué entre la sortie du four à induction et l'introduction dans la presse à filer.

5. Procédé de fabrication du cylindre haute pression sans jointures en acier inoxydable selon l'une des revendications 1 à 4, **caractérisé en ce que** pendant la première étape de fabrication, au cours de perforation, en poussant l'outil (7) de perforation sur le découpage (1), le revêtement (2) en matériau à base de verre soluble se casse et s'écaille au cours de processus de filage par la presse à filer jusqu'à ce qu'au moins la majeur partie en soit éliminé.

6. Procédé de fabrication du cylindre haute pression sans jointures en acier inoxydable selon la revendication 5, **caractérisé en ce qu'après** l'obtention de la forme finale du cylindre à partir du semi-produit (5), les résidus de revêtement (2) à base de verre soluble sont éliminés de la surface du semi-produit (5) en utilisant le soufflage sous pression de sa surface extérieure ainsi que de sa surface intérieure.

7. Procédé de fabrication du cylindre haute pression sans jointures en acier inoxydable selon l'une des revendications 1 à 6, **caractérisé en ce que** le découpage (1) est fabriqué en acier inoxydable, le cylindre finale est façonné sous la forme d'un cylindre sans jointures dont le volume peut aller de 5 à 260 litres, pour n'importe quel volume se situant sur la plage indiquée, comme à un goulot ou à deux goulots.

8. Procédé de fabrication du cylindre haute pression sans jointures en acier inoxydable selon la revendication 7, **caractérisé en ce que** pendant la seconde étape de fabrication, la paroi du semi-produit (5) est façonnée de manière à ce que son épaisseur soit de 2 à 21,5 mm.
